

## UNITED STATES PATENT OFFICE

2,287,712

## FERROTITANIUM ALLOY

Jerome Strauss, New York, N. Y., and Holbert Earl Dunn, Bridgeville, Pa., assignors to Vanadium Corporation of America, New York, N. Y., a corporation of Delaware

No Drawing. Application February 15, 1940,  
Serial No. 319,080

3 Claims. (CL. 75—58)

This invention relates to ferro-titanium alloys useful as addition agents for iron and steel. It relates more particularly to ferro-titanium alloys containing a substantial amount of manganese. The presence of manganese in substantial amount in these ferro-titanium alloys results in dense brilliant alloys free from slag inclusions, oxide and nitride products. The alloy containing a substantial amount of manganese appears to render easier the removal of the products of deoxidation of the steel or of other non-metallic particles with which these deoxidation products may associate themselves. The resultant steel is, therefore, cleaner and there is less likelihood of defective articles resulting from the presence of non-metallic particles during hot or cold working or machining, that would be disadvantageous either to the mechanical properties or to the surface appearance of the finished articles.

The present application is a continuation-in-part of application Serial No. 306,179, filed November 25, 1939, which in turn is a continuation-in-part of application Serial No. 114,830, filed December 8, 1936.

Ferro-titanium alloys according to the present invention may be of the low, medium or high carbon types. Ferro-titanium alloys containing under .5% carbon are generally classified as low carbon ferro-titanium, those containing from .5 to 5% carbon as medium carbon ferro-titanium, and those containing over 5% carbon as high carbon ferro-titanium. In our alloy, the carbon is less than 10% and preferably is between .05 and 8%. The titanium may be as low as 10% or as high as 50% by weight of the alloy but is preferably between about 15 and 45% or more particularly between about 15 and 30%. The alloy also contains manganese in substantial amount or both manganese in substantial amount and silicon. The manganese amounts to about 2 to 15% of our alloy, the preferred range being from about 3 to 10% or more, particularly from about 4 to 7%.

Our alloy may or may not contain substantial amounts of silicon or aluminum or both silicon and aluminum in addition to the iron, carbon, titanium and manganese. Where silicon is present in the alloy, it may amount to about .05 to 30% or preferably from about 1 to 15%. In the manufacture of low, medium and high carbon ferro-titanium alloys, silicon often is present in amounts ranging from less than 1% up to about 4%, depending upon the starting materials and the particular method employed. In the

manufacture of low and medium carbon ferro-titanium alloys, silicon is sometimes present in amounts between about 10 and 20%. Similarly some aluminum is always present in ferro-titanium alloys. Medium and high carbon ferro-titanium alloys may contain aluminum in amounts from a trace up to about 3%, depending upon the nature of the raw materials which are employed. Low carbon ferro-titanium alloys produced by methods using aluminum as the reducing agent may contain up to about 10% of aluminum. Our invention covers ferro-titanium alloys in which there is a substantial amount of manganese and in which silicon or aluminum or both may or may not be present. The silicon in our alloy may be up to about 30% and the aluminum may be up to about 10%. Our alloy containing manganese within the ranges specified is advantageous over the prior known ferro-titanium alloys whether or not our alloy contains a substantial amount of silicon. For certain purposes, the presence of substantial amounts of silicon or aluminum or both silicon and aluminum content may be employed in the alloy. Substantial amounts of manganese imparts further advantageous properties to the alloy. Our ferro-titanium alloy always contains at least 20% of iron, and in the preferred compositions contains at least 40 or 50% of iron.

We have discovered that part of the titanium content of the ferro-titanium may be effectively replaced by zirconium. The amount of zirconium should not in any case be greater than 50% of the titanium plus zirconium content. In other words, the amount of zirconium should not exceed the amount of titanium. Any amount of zirconium up to an amount equal to the titanium content may be employed in the alloy, although we prefer that the zirconium be from 15 to 50% of the titanium. A very useful alloy, for example, contained:

|                                | Per cent |
|--------------------------------|----------|
| C                              | 4.0      |
| Si                             | 3.5      |
| Mn                             | 6.5      |
| Ti                             | 17.5     |
| Zr                             | 5.0      |
| Balance substantially all iron |          |

We have used with greatest success alloys in which the manganese was in the range of about 10 to 40% of the content of titanium where the alloy does not contain an appreciable amount of zirconium, or a range of about 10 to 40% of the content of titanium plus zirconium where the alloy contains an appreciable amount of zirco-

nium, regardless of whether the manganese was employed alone or together with silicon.

We have found that the addition to steels or irons of a ferro-titanium alloy containing manganese or both manganese and silicon within the ranges specified produces effects in respect to cleanliness, soundness and uniform crystallization in the irons and steels which are markedly different from those obtained when the ferro-alloys of these elements are used independently. In other words, the use of this ferro-titanium alloy containing manganese or both manganese and silicon, either with or without zirconium present, produces results in steel deoxidation and cleanliness that are not obtainable by the addition of the separate ferro-alloys when added to steel either simultaneously or successively. In fact, steels treated with the alloys of this invention are found to be free from nitrogen containing inclusions that so frequently occur in steels to which have been added the titanium or zirconium alloys heretofore known.

A major field of application of ferro-titanium alloys according to the present invention, especially the medium carbon ferro-titanium alloys containing from .5 to 5% carbon, is in deoxidizing the so-called "rimmed" steels which require an ingot surface of the highest attainable quality. For this purpose, it is customary to treat the liquid steel in the ladle with from 1 to 3 pounds of ferro-titanium per ton or 0.01% to 0.03% titanium in the steel were the titanium recovered 100%. As a matter of fact, only traces of titanium can usually be found residual in the solidified steel, the bulk of the addition having reacted with and been slagged off with the ferrous oxide, manganese oxide, nitrides and silica particles entrained or dissolved in or precipitated during cooling from the molten metal. If for example, 3 pounds of ferro-titanium alloy are added per ton of steel, the alloy having an analysis of 20% titanium, 6% manganese, 3% silicon and 4% carbon, and these elements are recovered 100%, the analysis of the steel would be changed to the extent of 0.03% titanium, 0.009% manganese, 0.005% silicon and 0.006% carbon. When sheet and tin bar are being produced at 0.05% to 0.08% carbon, the possibility of carbon, manganese and silicon pick-up caused by deoxidizer additions is of importance. As a matter of fact, this "pick-up" is rarely observed within the range of ordinary analytical methods, as part of these reducing agents are oxidized by the ferrous and other oxide content of the molten steel and slagged off, while the amounts remaining are less than the sensitivity of the analytical methods.

In the high carbon or "killed" steels, where high-carbon or medium-carbon ferro-titanium additions as high as 18 pounds per ton have been made, the analysis of the steel, in case 100% recovery of the alloying elements added in the ferro-titanium deoxidizer could be effected, would only be changed to the extent of 0.12% titanium, 0.05% manganese, 0.03% silicon, and 0.036% carbon, for the maximum addition. In practice, 10 much less than 100% recovery and usually no recovery of these elements other than carbon, is experienced, as is the case in treating lower carbon steels. Moreover, the analysis of the untreated steel can be adjusted to allow for the 15 actual pick-up of this carbon.

The ferro-titanium alloys of the present invention may be made by any suitable process. The process disclosed in the above mentioned applications, Serial Nos 114,830 and 306,179, provides a very convenient way of producing the ferro-titanium alloys, particularly those containing 20 a medium carbon content.

The invention is not limited to the preferred 25 embodiments but may be otherwise embodied or practiced within the scope of the following claims.

We claim:

1. A ferro-titanium alloy containing less than 30 10% carbon, an effective amount of titanium, an effective amount of zirconium, the sum of the titanium and zirconium being between about 10 and 50%, the zirconium not exceeding the titanium, about 2 to 15% of manganese, the balance being substantially all iron except for silicon in 35 amount from about .05 to 30% and aluminum in amount from a trace up to about 10%.

2. A ferro-titanium alloy containing less than 40 10% carbon, an effective amount of titanium, an effective amount of zirconium, the sum of the titanium and zirconium being between about 10 and 50%, the zirconium not exceeding the titanium, about 3 to 10% of manganese, the balance being substantially all iron except for silicon in 45 amount from about .05 to 30% and aluminum in amount from a trace up to about 10%.

3. A ferro-titanium alloy containing less than 50 10% carbon, an effective amount of titanium, an effective amount of zirconium, the sum of the titanium and zirconium being between about 10 and 50%, the zirconium being about 15 to 50% of the titanium, about 2 to 15% of manganese, the balance being substantially all iron except for silicon in amount from about .05 to 30% and aluminum in amount from a trace up to about 55 10%.

JEROME STRAUSS.  
HOLBERT EARL DUNN.

CERTIFICATE OF CORRECTION.

Patent No. 2,287,712.

June 23, 1942.

JEROME STRAUSS, ET AL.

It is hereby certified that error appears in the printed specification of the above numbered patent requiring correction as follows: Page 1, second column, lines 23 and 24, for "aluminium content may be employed in the alloy," read --aluminum in our ferro-titanium alloys containing--; and that the said Letters Patent should be read with this correction therein that the same may conform to the record of the case in the Patent Office.

Signed and sealed this 4th day of August, A. D. 1942.

Henry Van Arsdale,

(Seal)

Acting Commissioner of Patents.